

C. H. SMITH.

## PROCESS OF TREATING COAL.

APPLICATION FILED JAN. 20, 1916.

1,276,427.

Patented Aug. 20, 1918.



**WITNESS**

WITNESS  
Geo. Schatz,  
M. F. Keating

Charles Howard Smith <sup>INVENTOR</sup>

Kiddle & Maagroon  
BY  
his ATTORNEYS

# UNITED STATES PATENT OFFICE.

CHARLES HOWARD SMITH, OF SHORT HILLS, NEW JERSEY, ASSIGNOR TO INTERNATIONAL COAL PRODUCTS CORPORATION, OF RICHMOND, VIRGINIA, A CORPORATION OF VIRGINIA.

## PROCESS OF TREATING COAL.

1,276,427.

Specification of Letters Patent. Patented Aug. 20, 1918.

Application filed January 20, 1916. Serial No. 73,108.

To all whom it may concern:

Be it known that I, CHARLES HOWARD SMITH, a citizen of the United States, and a resident of Short Hills, in the State of New Jersey, have invented a new and Improved Process of Treating Coal, of which the following is a specification.

My invention relates to a new and useful process of treating solid fuels, such as coal, which soften on heating, and to the resulting products which are recovered from said fuels by the carrying out of said process:

Some of the objects of my invention are:

- (1) A continuous process of heating coal so as to distil off some of the volatile substances contained therein and change the coal or solid fuel to a plastic condition;
- (2) to subject coal to a relatively low heating, thus placing in suspension the air, moisture, gases and vapors which are produced at low temperatures, then carrying the heat to a higher point so as to produce in a state of vapor or gas other substances which do not pass to the state of vapor or gas at lower temperatures, utilizing this property of some of the constituents to dilute and wash out the gases and vapors produced at lower temperatures;
- (3) to regulate and control the pressure of the gases within the retort and their passage through the condensing and purifying apparatus by means of an exhauster;
- (4) to regulate and control the heat in all parts of the apparatus in which the coal is heated so that the total heat applied during the period of its application is less than the amount required for ultimate destructive distillation during such period;
- (5) to prevent the access of sufficient air into the retort while the distillation is taking place to produce combustion within the retort and raise the temperature sufficiently to produce coke;
- (6) to discharge the residual mass while still in the plastic condition from the retort;
- (7) to subject the residual mass to a partial compression prior to subjecting it to final compression in order to exclude some of the entrained gases and prevent the occlusion of air when the mass is exposed to the air;
- (8) to introduce an admixture of either partially distilled coal or coke throughout the plastic material prior to final compression;
- (9) to lower the tem-

perature of the residual mass by the introduction of this admixture;

- (10) to absorb by this unsaturated admixture any remaining entrained gases or condensates within the plastic mass;
- (11) to then form the entire mass into briquets;
- (12) to provide suitable means of conveying the material from the retort to the presses without undue exposure to the air;
- (13) to cool slowly the hot briquets to the atmospheric temperature;
- (14) to recover the by-products from the coal distilled within the retort;
- (15) to produce a denatured fuel of uniform size approximating in physical and chemical qualities a natural coal of substantially the same volatile content when compared on an equal ash basis;
- (16) to produce a briquet having a fuel value different from the raw coal or fuel from which it is made but having substantially the same fuel value as a coal of equal ash and equal volatile content;
- (17) to produce a substantially tarless fuel of particular value for certain purposes;
- (18) to recover some of the more valuable constituents contained in the coal without reducing its fuel value per pound of fuel by elimination of the volatile ingredients most conducive to the formation of smoke;
- (19) to produce a fuel composed either of coal and partially distilled coal or coke and partially distilled coal.

Heretofore in processes which have been attempted for treating solid fuels such as coal for the purpose of converting the same into briquets, it has been found that the resultant product or briquets have been of little commercial value due to the brittleness of the briquets, thereby militating against their shipment. Such brittleness is due to a number of causes such as the compression of entrained gases in the residual mass at the time of compression; also due to the condensation of the volatile substances on the surface of the individual particles of the residual mass prior to compression, this condensation interfering with coherence between the particles when under compression; also to the imperfect cooling following the briquetting. By my improved process, I remove or eliminate these entrained gases from the plastic heated mass after it passes from the retort. Some of

these gases are condensed or driven back into the retort by partial compression, the remainder are absorbed by the introduction of a percentage of either partially distilled coal, or coke, introduced throughout the 5 mass and possessing a power of absorbing any entrained gases or condensates remaining in the plastic material as the temperatures of the two materials equalize. I then 10 compress the residual mass into briquets of suitable shape or size without the further admixture of a binder, and properly cool the briquet through the stages subsequently thereto.

15 The process may be best described with reference to an apparatus for carrying out said process, this apparatus and the various steps of the process being illustrated diagrammatically in the accompanying drawing, in which the figure represents a typical 20 apparatus for carrying out the process.

Referring to the drawing B represents a crusher of the usual type adapted to crush or pulverize coal A; C an elevator to elevate the coal to the hopper D; E a spout which feeds the coal to the stoker F. The 25 stoker F is provided with suitable means, such as a plunger for conveying the coal into the retort G, located within the furnace H. The furnace H is provided with means, such as an arch-shaped heating chamber, below which is located a bed of refractory material and suitable gas and 30 hot air burners, arranged to heat the retort G uniformly.

The retort G is provided with a mixer and conveyer J, located therein, the retort and mixer being so constructed and arranged that the coal within the retort G is mixed, 35 distilled, passed through, and continuously delivered from the retort G. The retort G is connected with the screw conveyer L by the hopper K. The screw conveyer L is so arranged and constructed that as the partially 40 distilled coal passes from the hopper K through the conveyer L, it first receives an admixture of either partially distilled coal, or coke, and thereafter undergoes partial compression, for the purpose mentioned 45 above.

The plastic coal is delivered from the screw conveyer L to the apron conveyer N through the chute M. This chute is provided with a gate T for sealing off the air 50 from entering the retort G at any time that the hopper K and conveyer L are not sealed with plastic material.

The conveyer N is inclosed to prevent exposure of the material to the atmosphere 55 and is connected to the feed box O of the briquetting press P. As the material passes through the briquetting press, it undergoes a final compression, the resulting product being briquets X, which may be of any desired size and shape. Suitable cooling

means Q are provided for slowly cooling the briquets X as they come from the briquetting press P.

In order to offset the resistance arising from the passage of the products of distillation through the condensing and purifying apparatus, and to balance the pressure of the gases and vapors within the retort, I provide an exhauster U connected to the hydraulic main V. The retort G should 70 be provided with a dome or riser, which is connected with the hydraulic main V for the receiving of the gases. As the coal in the retort is subjected to gradually increasing temperatures the various gases and vapors developed at the lower temperatures are 75 swept out by the further evolution of gases and vapors produced only at higher temperatures, whereby the procedure may be carried out as a continuous process.

The gaseous products and vapors which are given off during the heating of the coal in the retort G pass off by their own pressure to the hydraulic main V, thence they are further conducted by the exhauster U 80 and separated by the usual condensing and distilling processes well known to those skilled in this art, into resulting by-products, including tar and oil products 1, ammonia 2, benzene and homologues 3, heating 85 gas 4 and commercial or illuminating gas 5. The heating gas is preferably utilized in my process for heating the retort G.

In carrying out my preferred process, the coal A is first crushed or pulverized in the 100 crusher B. From this crusher the coal is fed through the elevator C to the hopper D, thence to the spout E, and then by the stoker F to the retort G in the furnace H. By 105 means of the mixer contained in the retort G the coal is distilled and conveyed through the retort. The heating is first at a relatively low temperature in order to expel the air and any gases, moisture and vapors which are produced at these temperatures. As the coal progresses through the retort 110 the heating is continued to a higher temperature so as to produce in a state of vapor or gas other substances in the coal which do not pass to the state of vapor or gas at the 115 lower temperatures, and to utilize these additional vapors and gases to dilute and wash out the gases and vapors produced at the lower temperatures. That is, by my process the temperature of the coal is raised progressively as it passes through the retort, thereby making it possible to utilize the properties of these additional vapors and 120 gases to dilute and wash out the vapors and gases produced at the lower temperatures.

If it is desired to secure fractional distillation, a series of retorts may be utilized, and each of these retorts being heated to a different degree of temperature, so that as the heated coal passes from one retort to the 125

next it will be subjected to the required varying temperatures to secure fractional distillation.

- While I have illustrated an apparatus comprising one retort, yet it is possible to carry out this fractional distillation by using either one retort or more than one, depending upon the degree to which it is desired to carry out fractional distillation.
- 10 But in any event, whether using a single retort or whether using a series of retorts, the total amount of heat applied to the coal during the period of its application must be less than the amount required for ultimate 15 destructive distillation in the same period.

It is also essential to prevent the access of air to the retort during the distillation in such quantities as will produce combustion sufficient to raise the temperature within the 20 retort to the point where coking will take place.

It will be found that the required amount of heating will depend upon the character of the coal treated for the reason that different coals must be heated to varying degrees of temperature in order to secure the desired results.

The gases and vapors which are given off while the coal is being heated are rich 30 in hydro-carbons. These gases and vapors pass off from the retort or retorts by their own pressure to the hydraulic main V and the subsequent resistance overcome by the exhauster U. They are then separated by 35 the usual condensing and distillation processes into gas for illuminating and heating purposes and into tar and oil products, ammonia and other by-products.

After the coal has been sufficiently heated, 40 it is forced into the hopper K and conveyed from the hopper K by the conveyer L. During this period of translation the heated material undergoes a partial compression and admixture with the material, such as 45 partially distilled coal or coke, in order to exclude and absorb any entrained gases.

The function of the conveyer N is to slightly further lower the temperature of the residual mass and to concentrate the 50 output of the one or more retorts at the feed box O ready for compression into briquets X.

In the feed box O the material from one or more retorts is suitably mixed and the residual mass fed to the briqueting press P 55 where it is subjected to the final compression so that the resulting briquet X will be sufficiently hard in structure for commercial shipment or use.

For further cooling to atmospheric temperature, I have provided suitable cooling means Q so that as the briquets are delivered from the press they will be cooled gradually before exposure to the air at atmospheric temperature.

65 In carrying out my process, I have found

that the finished product or briquet, which may be of any desired shape or size, approximates in burning qualities a natural coal having substantially equal ash and equal volatile content. While this resulting 70 briquet has a fuel value different from the raw coal from which it is made, yet it has substantially the same fuel value as raw coal having equal ash and equal volatile content.

By my process it is not essential to introduce a binder into the material before or while it is being briqueted, the plastic portion of the material containing sufficient binding qualities for the entire mass. In 80 my process the heat in all parts of the apparatus in which the coal is heated should be regulated and controlled so that the heat applied during the process and the period of its application is less than the amount required for ultimate destructive distillation.

The ultimate percentage of volatile matters or hydro-carbons can be controlled within a considerable range by my process so as to vary the character of the briquets and 90 by-products as desired.

By my process the relative quantities of the constituents of the raw coal are changed by low temperature distillation and limited carbonization, so that the resultant product, 95 after it has been briqueted, is a dense, hard, denatured fuel, comparing favorably with coal having equal ash and equal volatile content suitable for commercial shipment. This density and hardness of the briquet are 100 due to the substantial removal, condensation, or absorption of some of the constituents of the coal in a gaseous state, which are either removed, solidified or absorbed prior to briqueting, and also due to the reduction to a 105 minimum of internal strains within the briquet.

The resultant product, substantially smokeless and tarless, is of particular merit where fuels of this character are required.

By the expression "ultimate destructive distillation" as used herein, I mean substantial elimination of all the volatile constituents of the coal.

While I have described the use of partially 115 distilled coal or coke, as the material to be mixed with the plastic coal, yet I do not wish to limit myself to the use of these materials only, for my invention comprises the admixture with the plastic coal of any combustible material which has the property of absorbing the residual gases and condensates contained in the material extruded from the retort before the same is pressed into the form of briquets.

Nor do I wish to limit myself to the admixture of said materials with the plastic coal after it has passed from the retort, for in my process the coke, or a material of similar characteristics may be intermixed 120 125 130

with the plastic coal at any time after the plastic coal—or the plastic coal residue as it may be called—has left the heating zone and carried through the remaining steps of 5 the process, with the same result of absorbing the residual gases and condensates in the plastic material.

What I claim is:

1. The process of forming briquets consisting in heating coal to a plastic condition, removing the coal while in said condition from the heat zone, partially compressing said removed coal and introducing into said plastic coal an admixture of combustible material which will absorb gases and condensates entrained in said plastic coal, and mixing and subsequently pressing into briquets said material while in a heated condition.
2. The process of forming briquets consisting in heating coal to a plastic condition and distilling gases therefrom, removing the coal residue while in said heated condition from the heat zone, subsequently introducing into said coal while in plastic condition an admixture of coke to absorb the gases and condensates entrained in said plastic coal and partially compressing said removed plastic coal residue, and mixing and subsequently pressing into briquets said heated coal residue and said coke while in heated condition.
3. The process of treating coal consisting in heating coal to a plastic condition, removing it from the zone in which it has been heated, then introducing into said plastic coal a combustible material which will absorb the gases and condensates entrained in said plastic coal, then partially compressing the mass and finally molding it into pressed briquets.
4. The process of treating coal consisting in heating coal to a plastic condition, removing it from the heat zone, then introducing into it and mixing therewith coke for the purpose of absorbing gases entrained in the coal, then partially pressing the mass and finally compressing and molding the mass into briquets.
5. The process of treating coal consisting in subjecting the coal to a series of varying temperatures so that the total amount of heat applied during the successive periods of its application is less than the amount required for the ultimate destructive distillation, removing said coal from the heat zone and introducing into said heated coal a combustible material for absorbing the gases and condensates contained in said coal,

subjecting the mixture to a partial compression and ultimately subjecting it to a final compression and molding it into briquets.

6. The process of treating coal consisting in heating coal to a plastic condition and while it is in said condition introducing 65 therein and mixing therewith a combustible material such as coke for the purpose of absorbing the gases and condensates entrained in said coal and also while in said condition subjecting the coal to a plastic compression, 70 and subjecting the mass when partially cooled to a final compression and molding it into briquets.

7. The process of treating coal consisting in heating coal in a manner to distil gases 75 therefrom and until the coal residue is in a plastic condition, removing the coal residue from the zone in which it has been heated, then introducing into said plastic coal residue a combustible material which will absorb gases and condensates entrained in said plastic residue, partially compressing the mass and finally molding into pressed briquets.

8. In the manufacture of briquets the 85 method which comprises heating coal in order to eliminate some of the volatile material contained in the coal and until there results a plastic coal residue, removing said plastic residue from the heating zone, thereafter 90 mixing therewith material for the purpose of absorbing gases and condensates entrained in said plastic residue and subjecting said plastic residue to a partial compression, and finally forming the resulting 95 mass into briquets by pressure.

9. In the manufacture of briquets the method which consists in heating coal in a manner to partially devolatilize the coal and until the resulting residue is in a plastic 100 condition, removing said residue from the heat zone and introducing therein and mixing therewith material such as coke for the purpose of absorbing gases and condensates entrained in said residue, subjecting said 105 residue while in plastic condition to a partial compression, allowing the mass resulting from the mixing of the coal residue and the coke to become partially cooled and finally subjecting the partially cooled mass 110 to a final compression during which the mass is molded into briquets.

This specification signed and witnessed this 18th day of January, 1916.

CHARLES HOWARD SMITH.  
Signed in the presence of—

G. MCGRANN,  
W. C. MARGESON.